

(Specimens.)

D. C. RIPLEY, A. H. HEISEY & G. B. SWIFT.

MANUFACTURE OF ORNAMENTAL GLASSWARE.

No. 331,824.

Patented Dec. 8, 1885.



Fig. 1.



Fig. 2.

*Witnesses.*

Harry L. Gill.  
M. S. Connor

*Inventors.*

Daniel C. Ripley  
Augustus H. Heisey  
George B. Swift  
by their atty  
Baker, Ellsworth

# UNITED STATES PATENT OFFICE.

DANIEL C. RIPLEY, AUGUSTUS H. HEISEY, AND GEORGE B. SWIFT, OF  
PITTSBURG, PENNSYLVANIA.

## MANUFACTURE OF ORNAMENTAL GLASSWARE.

SPECIFICATION forming part of Letters Patent No. 331,824, dated December 8, 1885.

Application filed September 21, 1885. Serial No. 177,662. (Specimens.)

*To all whom it may concern:*

Be it known that we, DANIEL C. RIPLEY, AUGUSTUS H. HEISEY, and GEORGE B. SWIFT, of Pittsburg, in the county of Allegheny and 5 State of Pennsylvania, have invented a new and useful Improvement in the Manufacture of Ornamental Glassware; and we do hereby declare the following to be a full, clear, and exact description thereof.

10 It has been customary in the manufacture of parti-colored glassware to cover the surface of the clear-glass article with a thin layer of colored glass by the process known to the glass trade as "flashing," and then to cut the de- 15 sired figure or pattern into the surface of the article through and below the colored surface-layer. The product of this process is one of the most expensive kind of glassware, for the reason that the operations of "flashing" and 20 "cutting" are both very expensive. Consequently this glassware is in but limited use, and is practically beyond the reach of persons of limited means.

25 The object of our invention is the production of an article of similar character and like appearance at a greatly reduced cost.

To enable others skilled in the art to make use of our invention, we will now describe it, reference being had to the accompanying 30 drawings, in which—

Figure 1 is a bottom view of a glass dish produced by our improved method, and Fig. 2 is a side view of the same.

Like letters of reference indicate like parts. 35 The dish *a* is pressed in a suitable mold, the inner face of which is cut with the design or pattern, which will produce the design which appears on the surface of the article, consisting of a series of grooves, *b*, crossing each 40 other at various angles, in imitation of a pattern produced by the operation of glass-cutting, and such as will leave a series of raised surfaces, *c*, of the shape shown, or of other shapes,

depending on the particular pattern selected. The raised or elevated surfaces are then coated 4 with a suitable coloring-matter or paint, leaving the grooves or depressed portions clear, and then the article is placed in a suitable oven or furnace, and the coloring-matter is baked in the manner practiced in baking 5 decorated plaques.

The pressing operation, if carefully conducted with clear sharp-cut molds, will produce articles so nearly resembling cut ware that the difference can only be detected by an 5 expert, and with a little care the application and baking-on of the color can be so perfectly done as to be indistinguishable by inspection of the article alone from flashed glass.

The cost of the whole operation is little, if any, greater than that of the flashing operation, and it produces a beautiful and salable article, which the manufacturer is able to sell at a price low enough to put it within the reach of persons of limited means who are 6 unable to afford the cut ware before referred to.

What we claim as our invention, and desire to secure by Letters Patent, is—

The method of making ornamental glassware, which consists in pressing a glass article with raised and depressed surfaces, in imitation of cut-glass patterns, painting the raised surfaces, and then baking in the color on the same, substantially as and for the purposes 7 described.

In testimony whereof we have hereunto set our hands this 2d day of September, A. D. 1885.

DANIEL C. RIPLEY.  
AUGUSTUS H. HEISEY.  
GEORGE B. SWIFT.

Witnesses:

W. B. CORWIN,  
THOMAS W. BAKEWELL.